

1

2,872,343

## METHOD OF PROTECTIVELY COATING URANIUM

Lowell D. Eubank, South Euclid, Ohio, and Ernest R. Boller, Marion, Ind., assignors to the United States of America as represented by the United States Atomic Energy Commission

No Drawing. Application March 14, 1946  
Serial No. 654,504

5 Claims. (Cl. 117—51)

This invention relates to the coating of metallic uranium. Coated metallic uranium articles are useful as fuel elements in neutronic reactors of the type described in the co-pending application of Fermi et al. Serial No. 568,904, filed December 19, 1944, now Patent No. 2,708,656, granted May 17, 1955.

Early attempts to coat metallic uranium with zinc met with unsatisfactory results because of the failure of the zinc to coat the metal uniformly. Coatings applied by dipping the metallic uranium into molten baths of zinc of the composition normally employed in the application of zinc coatings to steel and similar metals resulted in only spotty coverage of the metallic uranium. In accordance with the teachings of our United States patent application Serial Number 588,060, filed April 12, 1945, now Patent No. 2,848,796, granted August 26, 1958, we have found that satisfactorily adherent coatings of zinc can be applied provided a substantial proportion of aluminum is present in the molten zinc so as to form a uranium-aluminum alloy layer between the metallic uranium and the zinc. For some purposes, the alloy coatings of zinc containing aluminum are as satisfactory as zinc coatings or superior to zinc coatings. For some purposes, however, the presence of aluminum is objectionable.

An object of the present invention is the provision of firmly adherent protective coatings on metallic uranium. A further object is the provision of such coatings suitable for use as bases for the application of other metal coatings. A yet further object of the invention is the provision of zinc coatings on metallic uranium without the use of substantial proportions of aluminum in the zinc coating alloy to provide a uranium-aluminum alloy interlayer.

In accordance with the present invention it has been discovered that by employing a zinc which is free from lead and iron impurities, continuous coatings of zinc on metallic uranium may be applied without the use of an aluminum alloy. Commercial zinc normally employed for the application of hot dip coatings may contain up to 1.6% of lead and up to 0.08% of iron. Such zinc compositions result in the spotty coatings previously referred to. We have found that by employing a zinc which contains less than 0.01% of lead and less than 0.01% of iron and preferably less than 0.01% total of lead, iron and cadmium, very uniform continuous coatings of zinc firmly adhering directly to the uranium may be applied.

The coatings of the invention provide very substantial protection for metallic uranium against the corrosive effects of the atmosphere and other active reagents.

For special purposes the zinc-coated uranium may be given a second coating with another metal more resistant to the corrosive influences particularly concerned. Thus coatings of lead containing a small proportion of silver or tin, or aluminum containing a minor proportion of silicon may be applied over the zinc coatings.

The coatings may be applied by dipping the uranium to be coated into a bath of zinc at a temperature between

2

about 430° C. and 600° C. The bath may be provided with a standard flux, preferably as alkali-metal chloride flux melting at substantially below bath temperature, or it may be devoid of flux.

5 The uranium may be prepared for coating by sandblasting or acid-pickling, preferably in warm strong nitric acid.

The following examples will illustrate the invention. Proportions are in terms of weight if not otherwise expressed.

## Example 1

A metallic uranium rod about two inches long and three-eighths of an inch in diameter was immersed in aqueous 50% HNO<sub>3</sub> solution at room temperature for about 5 minutes to clean the metal surface and rinsed in water. The rod was then dipped for 30 seconds into a bath of pure zinc containing less than 0.007% lead, less than 0.005% iron, less than 0.005% cadmium, and more than 99.99% zinc. The zinc bath was at a temperature of 540° C. and was covered with a molten flux comprising 37% lithium chloride, 53% potassium chloride and 10% sodium chloride. The metal rod was withdrawn from the molten zinc bath, shaken to free it from excess metal, and placed on "Transite" rolls rotating slowly until the coating solidified by normal cooling. When the coating had solidified, the rod was removed from the rolls and quenched in water. A smooth uniform coating of zinc over the entire surface of the metal and adhering directly to the uranium was thus obtained.

## Example 2

Five metallic uranium rods were cleaned in 50% nitric acid solution as described in Example 1 and dipped into molten zinc baths of the same composition as employed in Example 1 using the same flux. The temperatures of the molten metal baths were 555° C., 505° C., 450° C., 440° C., and 433° C. In each case a uniform, continuous coating of the zinc directly on the metallic uranium was obtained.

When an attempt was made to coat metallic uranium with an ordinary hot dip coating zinc (Prime Western Spelter) under the conditions described in this example, only spotty coatings could be obtained. Portions of the metallic uranium surface remained exposed after the coating operation in every case.

The following examples illustrate the application of multiple coatings employing a zinc coating as base.

## Example 3

50 A metallic uranium rod, coated as described in Example 1, was dipped in a molten bath containing 90% lead and 10% tin at 350° C. The lead-tin bath was protected by a flux comprising 27% ammonium chloride and 73% zinc chloride. The rod was immediately withdrawn from the molten metal bath and rolled on carbon rolls to solidify the coating. The uranium rod was uniformly coated with a continuous coating of lead-tin composition over a continuous separating coating of zinc.

## Example 4

60 A metallic uranium rod, after cleaning in aqueous 50% nitric acid solution, was dipped for 30 seconds in a zinc bath of the composition employed in Example 1, maintained at 560° C. and covered with a 37% lithium chloride, 53% potassium chloride, 10% sodium chloride flux. The rod was withdrawn from the bath, cooled in air for 10 seconds, and then rolled on "Transite" rolls until the coating solidified. The coated rod was quenched by immersion in water. The resulting rod, which was uniformly coated with zinc, was then dipped for 30 seconds into a molten lead bath comprising 98% lead and 2%

silver. The lead bath was covered with a flux containing 73% zinc chloride and 27% ammonium chloride. After 30 seconds in this bath the rod was withdrawn and rolled on "Transite" rolls until the coating solidified. It was then quenched by plunging it into water. A smoothly coated rod of metallic uranium was obtained with a composite coating of zinc followed by a thin zinc-silver layer and a final lead-silver layer.

*Example 5*

A metallic uranium rod prepared for coating as described in Example 1 was dipped for 1½ minutes in a zinc bath maintained at 500° to 510° C. The zinc bath was of the same high purity as employed in Example 1. After 1½ minutes in this bath the rod was removed and centrifuged for 8 seconds at 640 revolutions per minute in a centrifuge in which it was suspended coaxially at a distance of about 6 inches from the axis of rotation. The rod was then dipped into a bath comprising 88% aluminum and 12% silicon at a temperature of 620–625° C. for between 10 and 15 seconds, removed and dipped for 3 seconds into a second aluminum-silicon bath of the same composition maintained at 585° C. The rod was withdrawn from this second bath, rolled for 15 seconds on "Transite" rolls and then quenched in water. The rod was completely coated with aluminum-silicon alloy over a thin zinc interlayer.

It will be understood that we intend to include variations and modifications of the invention and that the preceding examples are illustrations only and in no wise to be construed as limitations upon the invention, the scope of which is defined in the appended claims, wherein we claim:

1. The method of protectively coating uranium, which comprises preparing the uranium for coating and dipping the freshly prepared metal into a bath of molten zinc containing less than 0.01% each of iron and lead, said bath being at a temperature between 430° C. and 600° C., withdrawing the uranium coated with zinc and cooling it to solidify the coating.

2. The method of protectively coating uranium, which comprises pickling the uranium in strong nitric acid and dipping the freshly prepared metal into a bath of molten zinc containing less than 0.01% each of iron and lead, said bath being at a temperature between 430° C. and 600° C., withdrawing the uranium coated with zinc and cooling it to solidify the coating.

3. The method of protectively coating uranium, which comprises pickling the uranium in strong nitric acid and dipping the freshly prepared metal into a bath of molten zinc containing less than 0.01% each of iron and lead,

4. said bath being at a temperature between 430° C. and 600° C., withdrawing the uranium coated with zinc, dipping the zinc-coated uranium into a molten bath comprising 88% aluminum and 12% silicon at a temperature of about 620–625° C. for just sufficient time to provide complete coating, withdrawing the coated uranium from the aluminum-silicon bath and cooling it to solidify the composite coating.

5. The method of protectively coating uranium, which comprises pickling the uranium in strong nitric acid and dipping the freshly prepared metal into a bath of molten zinc containing less than 0.01% each of iron and lead, said bath being at a temperature between 430° C. and 600° C., withdrawing the uranium coated with zinc, dipping the zinc-coated uranium into a molten bath comprising approximately 90% lead and 10% tin at a temperature of approximately 350° C. withdrawing the coated uranium and cooling it to solidify the composite coating.

6. The method of protectively coating uranium, which comprises pickling the uranium in strong nitric acid and dipping the freshly prepared metal into a bath of molten zinc containing less than 0.01% each of iron and lead, said bath being at a temperature between 430° C. and 600° C., withdrawing the uranium coated with zinc, dipping the zinc-coated uranium into a molten bath comprising approximately 98% lead and 2% silver, said bath being at a temperature below the melting point of zinc, withdrawing the coated uranium and cooling it to solidify the composite coating.

30

References Cited in the file of this patent

UNITED STATES PATENTS

|    |           |                  |               |
|----|-----------|------------------|---------------|
| 35 | 547,381   | McKnight         | Oct. 1, 1895  |
|    | 927,372   | Monnot           | July 6, 1909  |
|    | 1,114,792 | Monnot           | Oct. 27, 1914 |
|    | 1,497,265 | Haas             | June 10, 1924 |
|    | 1,597,189 | Gero             | Aug. 24, 1926 |
|    | 1,869,784 | Theiss           | Aug. 2, 1932  |
| 40 | 1,982,563 | Wimmer           | Nov. 27, 1934 |
|    | 2,231,967 | Tainton          | Feb. 18, 1941 |
|    | 2,276,101 | Schueler         | Mar. 10, 1942 |
|    | 2,299,166 | Miller           | Oct. 20, 1942 |
| 45 | 2,307,243 | Slagle           | Jan. 5, 1943  |
|    | 2,396,730 | Whitfield et al. | Mar. 19, 1946 |

OTHER REFERENCES

Metals Handbook, 1939 edition, page 1736.  
Protective Coatings for Metals, Burns and Schuh, 1939, 50 pages 60, 61, 64, 65, 94 and 101.